

## UNITED STATES PATENT OFFICE

JOHN A. GANN AND WILLIAM H. GROSS, OF MIDLAND, MICHIGAN, ASSIGNEES TO THE DOW CHEMICAL COMPANY, OF MIDLAND, MICHIGAN, A CORPORATION OF MICHIGAN

## METHOD OF TREATING MAGNESIUM AND PRODUCT OBTAINED THEREBY

No Drawing.

Application filed May 8, 1931. Serial No. 536,084.

The present invention relates to a process for coloring magnesium and magnesium alloy articles. Specifically, it deals with the treatment of such light metal articles with a 5 solution of a material having combined coloring and etching properties or with a solution of a material having coloring properties, but insufficient etching properties, to which is added another material, in relatively small 10 amount, having etching properties.

It has heretofore been proposed to treat a magnesium article with an emulsion of soap, oil, and water (United States Patent 1,477,- 922) to form a substantially colorless aliphatic soap base coating thereon which can be dyed if desired. It has also been proposed (United States Patent 1,480,869) to color magnesium and magnesium base alloy articles with a nitric acid solution containing either chromic acid or sodium bichromate and a salt of a heavy metal. We have now found that chromic acid, bichromates and other heavy metal compounds are unnecessary additions to a solution used for coloring magnesium articles. 20 We have also found that it is unnecessary to form a soap base coating on the article before it can be colored. We have further found that materials of an organic aromatic 25 nature can be used in an etching solution for coloring magnesium articles in a much more satisfactory manner than heavy metal compounds due partially to the fact that treatment with an etching solution of them suffi- 30 fices for the complete coloring treatment and a much greater range of colors can be obtained thereby. Accordingly, the principal object of the present invention is the provision of a method of coloring magnesium and 35 magnesium alloy articles by means of a coloring and etching bath containing an organic aromatic coloring agent for magnesium. Further objects and advantages will appear 40 as the description proceeds.

To the accomplishment of the foregoing and related ends, the invention, then, consists of the steps hereinafter fully described and particularly pointed out in the claims, the following description setting forth in detail 45 several modes of carrying out the inven-

tion, such disclosed modes illustrating, however, but several of various ways in which the principle of the invention may be used.

Our tests show that colored magnesium and magnesium alloy articles can be readily produced by subjecting the article to a bath containing an organic aromatic coloring agent of etching nature or an organic aromatic coloring agent, having insufficient etching action, in combination with a material in relatively small amount that will provide the etching action on the metal. For instance, in the case of articles made from magnesium and its alloys, picric acid has been found to have the property of etching, coating, and coloring the same. The coating formed, which may vary in color from a pale yellow to a black according to the treatment given, moreover, offers a certain amount of resistance to corrosion. The shade of the color, where picric acid is used, is influenced by the strength of the solution (solubility 6.3 per cent in water at 100° C.) and its temperature as well as the length of time the article is treated or immersed in it, and the 55 alloy used. Diphenyl sulphonic acid (para-phenyl-benzene-sulphonic acid) likewise has the property of coating, coloring, and etching the magnesium article without the aid of additional etchants. A magnesium-aluminum-manganese alloy article treated in a solution of this material takes on a semi-white coloration. A coating applied on the metal by treatment with diphenyl sulphonic acid acts not only to change the surface appearance of the article, but also gives some protection from corrosion and is a paint base. On the other hand, naphthol yellow, Bismarck brown, aniline red, malachite green-hydrochloride, Congo red, quinoline yellow, acid 60 fuchsine, alizarin blue, and the like, are preferably used in a solution having an etchant added thereto. Such etchant may be an acid, an ammonium salt, or other material having the property of attacking magnesium metal. 65 As a typical strong acid for use in the manner described we have found that a weak solution of hydrochloric acid is satisfactory. We have also used sulfanilic acid, which is a weak acid, with satisfactory results. On 70 75 80 85 90 95 100

the other hand, ammonium chloride is a typical ammonium salt for use in the manner described, and sodium bisulphate is a suitable acid salt for use in etching the magnesium article. Where strong acids are used, we have found that a solution containing up to  $\frac{1}{2}$  of 1 per cent of the acid is sufficient for most purposes,  $\frac{1}{16}$  of 1 per cent being normally the preferred amount. Where weaker acids are used, they will have to be used in higher concentrations to obtain an equivalent hydrogen ion concentration in the solution. On the other hand, where using ammonium salts, ammonium chloride is satisfactory and may be present in the solution up to 5 per cent. The preferred amount found satisfactory for most purposes is  $\frac{1}{2}$  of 1 per cent. While we have given preferred amounts and specific ranges for these materials, we do not wish to be limited to those exact amounts since, obviously, other amounts could be used in equivalent manner so long as the final effect is equivalent to that described. It is further to be noted that while we normally prefer to use an aqueous solution of the coloring and etching solution, at least part of the water can be replaced with other solvents such as alcohol. The terminology "etching solution" as used herein is to be understood to cover not only a solution of a material having both coloring and etching properties, but also a solution of a coloring material to which an etchant of the type described has been added.

The use of the aromatic coloring materials noted above, which are typical of their classes, permits a large range of colors to be obtained on the articles being treated, such colors ranging from semi-white through yellow, brass, green, red, brown, and black. In any case it will be understood that the particular color obtained will depend upon a number of variables, for instance, at higher temperatures the action is accelerated so that a shorter time will be required to obtain a given color for the same concentration of solution. The degree of concentration of the solution up to its saturation point also affects the coloring since with stronger solutions the action is faster. The coloring material in the solvent may be present, if desired, in an amount in excess of its solubility therein, and will thus be available to go into solution as fast as the dissolved material is used up in treating the magnesium articles. The color will also vary with the dye used. Where an etching material is used in the solution it also affects the color to a certain extent. The particular alloy treated will likewise have some influence on the coloring. For instance, where an aqueous solution containing  $\frac{1}{16}$  of 1 per cent of quinoline yellow and  $\frac{1}{16}$  of 1 per cent of ammonium chloride is used to treat a copper-containing magnesium alloy article, for instance, a mag-

nesium alloy containing 4 per cent copper, 2 per cent aluminum, 2 per cent cadmium, and .2 per cent of manganese, the ultimate coat obtained is an olive green when the treatment is carried out at 90° to 100° C. for 10 minutes. On the other hand, a yellow color is obtained under the same conditions where a copper-free alloy such as a magnesium alloy containing 4 per cent aluminum and .25 per cent manganese is used.

To set forth the invention in concise terms the following examples are given:—

#### EXAMPLE 1

*Brass coloring on a Dowmetal F alloy consisting of magnesium containing 4 per cent aluminum and .25 per cent manganese*

The article to be colored is first cleaned so as to be free from surface inclusions and contaminations and is then suspended in a bath which is composed as follows:—3 per cent picric acid, 97 per cent water. While the temperature of the bath may be substantially room temperature, we prefer to use a temperature of from 90° to 100° C., at which temperature 5 to 15 seconds suffice to bring out the brass coloring. The time, of course, may be varied from this to obtain the exact shade of color desired. During the treatment we prefer to frequently move the article or stir the bath so that any gas bubbles adhering to its surface will be dislodged and thus permit a uniform coloring over the entire surface of the article. At the completion of the treatment the article is quickly removed from the solution and washed with water, preferably hot water which facilitates the quick drying of the article.

The following examples relate to the coloring of the above noted Dowmetal alloy to obtain several other colors:—

#### EXAMPLE 2

*Brownish black coloring*

3 per cent picric acid, 97 per cent water. The solution is preferably heated to a temperature of 90° to 100° C. and the article agitated therein for 10 to 15 minutes, following which it is quickly removed and washed.

#### EXAMPLE 3

*Yellowish green coloring*

$\frac{1}{16}$  of 1 per cent water-soluble quinoline yellow,  $\frac{1}{16}$  of 1 per cent ammonium chloride, 99.8 per cent water. The bath is preferably heated to a temperature of 90° to 100° C. and the article agitated therein for 30 to 40 minutes, following which it is quickly removed and washed.

## EXAMPLE 4

## Gray coloring

5  $\frac{1}{10}$  of 1 per cent malachite green-hydrochloride,  $\frac{1}{10}$  of 1 per cent ammonium chloride, 99.8 per cent water. The cleaned Dowmetal to be coated is agitated in the solution at a temperature of 90° to 100° C. for 15 to 20 minutes, following which it is quickly removed and washed.

## EXAMPLE 5

## Brown coloring

15  $\frac{1}{10}$  of 1 per cent naphthol yellow S and  $\frac{1}{2}$  of 1 per cent of sulphanilic acid, 99.4 per cent water. The cleaned article is agitated for 5 minutes in the solution at a temperature of 90° to 100° C., following which it is quickly removed and washed.

The so colored articles after being dried can be treated with a coat of lacquer or spirit varnish to further aid in preventing corrosion of the article or to retain the color obtained by the treatment as well as overcome discoloration due to abrasion. The article, on the other hand, may have paint applied thereto in the conventional manner. Such materials when applied to the surface of magnesium articles will be hereinafter referred to as a protective coating.

While we have described our invention in terms of treating articles of magnesium and alloys thereof (specifically Dowmetal F) it is to be understood that the use of the term "magnesium" is intended to cover both magnesium and its alloys.

40 Picric acid, diphenyl sulphonic acid, and the other coloring materials, which we have described as suitable for coloring and otherwise favorably affecting the surface of magnesium articles, are typical of the various classes from which they are selected. These materials, moreover, are all organic aromatic 45 compounds well known to those familiar with the dye art. Accordingly, since such materials, as a class, act as coloring agents on magnesium, they will be referred to generically in the claims as organic aromatic coloring 50 agents for magnesium.

Other modes of applying the principle of our invention may be employed instead of those explained, change being made as regards the process herein disclosed, provided 55 the means stated by any of the following claims or the equivalent of such stated means be employed.

We therefore particularly point out and distinctly claim as our invention:—

60 1. The method of treating a magnesium article which comprises subjecting said article to the action of an etching solution containing an organic aromatic coloring agent for magnesium.

65 2. The method of treating a magnesium

article, which comprises subjecting same at a temperature of 90° to 100° C. to the action of an etching solution of an organic aromatic coloring agent for magnesium.

3. The method of treating a magnesium article, which comprises subjecting same to the action of an etching solution of one of the materials picric acid, diphenyl sulphonic acid, naphthol yellow, Bismarck brown, aniline red, malachite green-hydrochloride, Congo red, quinoline yellow, acid fuchsine, alizarin blue.

4. The method of treating a magnesium article, which comprises subjecting same at a temperature of 90° to 100° C. to the action of an etching solution of one of the materials picric acid, diphenyl sulphonic acid, naphthol yellow, Bismarck brown, aniline red, malachite green-hydrochloride, Congo red, quinoline yellow, acid fuchsine, alizarin blue.

5. The method of coloring a magnesium article, which comprises subjecting same to the action of an etching solution of an organic aromatic coloring agent for magnesium.

6. The method of coloring a magnesium article, which comprises the steps of cleaning said article with an acid solution, and treating it with an etching bath containing an organic aromatic coloring agent for magnesium.

7. The method of coloring a magnesium article, which comprises the steps of cleaning said article with an acid solution, treating it with an etching bath containing an organic aromatic coloring agent for magnesium, and thereupon washing and drying the article.

8. The method of coloring magnesium and magnesium alloy articles, which comprises subjecting same to the action of an etching solution of an acid type of organic aromatic coloring agent for magnesium.

9. The method of coloring magnesium and magnesium alloy articles which comprises subjecting same to the action of a solution of picric acid.

10. The method of coloring magnesium and magnesium alloy articles which consists in subjecting same to the action of an aqueous solution containing picric acid in amount up to its solubility therein.

11. The method of providing a magnesium or magnesium alloy article with a brass color, which consists in cleaning the article with an acid solution, thereupon agitating it in an aqueous solution of picric acid at a temperature of 90° to 100° C. and as soon as the required coloration has been obtained quickly rinsing it in water, and drying the article.

12. The method of coloring magnesium and magnesium alloy articles, which comprises subjecting same to the action of a solution of diphenyl sulphonic acid.

13. The method of coloring magnesium

and magnesium alloy articles, which comprises subjecting same at a temperature of 90° to 100° C. to the action of an aqueous solution containing diphenyl sulphonic acid in amount up to its solubility therein.

14. The method of coloring magnesium and magnesium alloy articles, which comprises subjecting same to the action of an etching solution of a basic type of organic aromatic coloring agent for magnesium.

15. The method of coloring magnesium and magnesium alloy articles, which comprises subjecting same to the action of an etching solution of malachite green-hydrochloride.

15. The method of coloring magnesium and magnesium alloy articles, which comprises subjecting same to the action of an etching aqueous solution containing malachite green-hydrochloride in amount up to its solubility therein.

17. The method of providing a magnesium or magnesium alloy article with a gray color, which consists in cleaning the article with an acid solution, thereupon agitating it in an aqueous solution of malachite green-hydrochloride and ammonium chloride at a temperature of 90° to 100° C. and as soon as the required coloration has been obtained quickly rinsing it in water, and drying the article.

18. A magnesium or magnesium alloy article provided with a closely adhering surface layer of a magnesium compound formed in place by the interaction of the magnesium with an etching solution of an organic aromatic coloring agent for magnesium.

19. A magnesium or magnesium alloy article provided with a closely adhering surface layer of a magnesium compound formed in place by the interaction of the magnesium with an etching solution of one of the materials picric acid, diphenyl sulphonic acid, naphthol yellow, Bismarck brown, aniline red, malachite green-hydrochloride, Congo red, quinoline yellow, acid fuchsine, alizarin blue.

20. A magnesium or magnesium alloy article provided with a closely adhering surface layer of a magnesium compound formed in place by the interaction of the magnesium with picric acid.

21. A magnesium or magnesium alloy article provided with a closely adhering surface layer of a magnesium compound formed in place by the interaction of the magnesium with diphenyl sulphonic acid.

22. A magnesium or magnesium alloy article provided with a closely adhering surface layer of a magnesium compound formed in place by the interaction of the magnesium with malachite green-hydrochloride.

Signed by us this 6th day of May, 1931.

JOHN A. GANN

WILLIAM H. GROSS.